

Oct. 16, 1923.

1,471,054

W. D. MOORE

ART OF PRODUCING CENTRIFUGAL CASTINGS WITH A PROTECTIVE COATING

Filed March 8, 1923

*Fig. 1.*



*Fig. 2.*



INVENTOR  
WILLIAM D. MOORE

BY  
Meyers, Cavanaugh & Whitehead  
ATTORNEYS

## UNITED STATES PATENT OFFICE.

WILLIAM D. MOORE, OF BIRMINGHAM, ALABAMA, ASSIGNOR TO AMERICAN CAST IRON PIPE COMPANY, OF BIRMINGHAM, ALABAMA, A CORPORATION OF GEORGIA.

## ART OF PRODUCING CENTRIFUGAL CASTINGS WITH A PROTECTIVE COATING.

Original application filed March 1, 1923, Serial No. 622,082. Divided and this application filed March 8, 1923. Serial No. 623,649.

*To all whom it may concern:*

Be it known that I, WILLIAM D. MOORE, a citizen of the United States, and resident of Birmingham, in the county of Jefferson and State of Alabama, have invented certain new and useful Improvements in the Art of Producing Centrifugal Castings with a Protective Coating, of which the following is a specification.

10 This invention relates to the art of centrifugally casting hollow metal bodies such as pipe, and more particularly to the making of such bodies in centrifugally operated refractory molds; and has special reference 15 to the provision of metal castings having outer protective coatings produced in the casting operation and to the method of making such castings, this application being a division of my application Serial No. 622, 20 filed March 1, 1923.

The principal objects of my present invention may be said to include the provision of a casting, and more particularly a centrifugally produced metal casting such 25 as ferrous pipe having a protective coating on its outer surface intimately united with the body of the casting for yielding a casting product which is capable of greatly resisting corrosive and other effects tending 30 to shorten the life of the pipe; the further provision of a centrifugally produced casting having a protective coating which is readily produced during the casting operation in an efficacious and economical manner, 35 and the provision of a method of producing the casting with the protective coating in a mold where the coating material is made to perform highly advantageous functions in the casting step for successfully permitting 40 the centrifugal casting on refractory and more particularly on "green" sand molds.

To the accomplishment of the foregoing and such other objects as may hereinafter appear, my invention consists in the elements and their relation one to the other, as hereinafter particularly described and sought to be defined in the claims, reference being had to the accompanying drawing showing a preferred embodiment of my invention, and in which:

Figure 1 is a cross-sectional view showing

a rotary or centrifugally operated mold of the refractory type provided with a facing which forms the coating of my invention, and

55 Figure 2 is a cross-sectional view of the rotary mold after a casting operation and showing the facing on the surface of the casting functioning as a protective coating therefor.

60 Before describing my invention in detail, I will premise that in producing the centrifugally made casting with the protective coating, I first line a rotary mold with a refractory and more particularly a "green" or moist sand lining, which lining is then faced with a powdered substance having the properties of absorbing moisture from the lining and of taking a quick initial set to produce a tough membranous coating or facing for the lining, and of being of a fusible character so as to fuse to the outer surface of the casting to provide therefor the desired protective coating.

65 In lining the mold I first preferably provide a sand mixture having preferably a moisture content sufficient to provide a bonding power for the mixture to withstand the cutting and washing action of the iron and insufficient to produce that objectionable amount of steam generation which in practice has been found to result in pocketed or honeycomb defects in the casting. The sand mixture I prefer to employ contains 50% of silicia sand, 35% of sharp sand, and 80 15% of molding sand, this mixture containing from 7% to 11% of uncombined water calculated on the weight of the dry sand, all as described and claimed in my co-pending application Serial No. 623,650, filed 85 March 8, 1923.

90 Referring now to Fig. 1 of the drawings, I show diagrammatically a mold comprising a flask 10 provided with a plurality of perforations 11 distributed over the body 95 thereof, these perforations defining vent holes for the gases and steam generated during the casting step, and this mold may be provided with a bell end 12 where pipe having a bell mouth end is desired to be 100 produced. This flask is first lined with a refractory lining 13 which in the preferred

practice of the invention comprises the moist sand mixture hereinbefore referred to.

As hereinbefore stated, it is a principal object of the present invention to produce 5 centrifugally cast hollow bodies such as ferrous pipe having an outer protective coating which is readily produced during the casting operation, the protective coating produced on the casting first forming a facing 10 for the refractory mold and having very desirable properties and functions as a facing for the refractory mold.

To accomplish these ends, I employ a facing material which is applied to the surface 15 of the moist sand mold in a powdered state, the powdered material having the properties of absorbing moisture from the sand lining 13, of taking a quick initial set to produce a tough membranous or skin-like mold facing 20 which is highly refractory, of having a low capacity for absorption of heat, of producing a mold wall impervious to the molten metal, and of being of a fusible nature so as to readily unite with the skin of the casting 25 to produce the desired protective coating therefor. I have discovered that such a facing is produced with the use of natural cement, this being a pulverized product resulting from the calcination of an argilla- 30 ceous limestone at a temperature only sufficient to drive off the carbon dioxide.

The powdered natural cement may be applied to the face of the moist sand mold by means of the apparatus disclosed and 35 claimed in my copending application Serial No. 587,999 filed Sept. 13, 1922, for a mold facing device. Immediately the application is made, the powdered cement begins to absorb moisture from the moist sand lining 13 40 and chemically reacts to quickly take an initial set, producing instead of a soft powdered face a rather tough membranous or shell-like facing indicated as 14 in Fig. 1 which has a high resistance to the cutting 45 action of the iron, which has the property of taking a quick initial set without any application of heat, and which upon setting expands with the result that the facing tends to pack itself or imbed itself into the sand 50 mold proper and in the grains of the sand on the face of the mold so as to become at this stage of the process practically an integral part of the mold, the effect including a conditioning of the sand lining for the 55 high resistance to destruction displayed thereby when molten metal is poured thereinto.

While in most instances I may employ natural cement in its natural state, in some 60 instances it is desirable to mix with the natural cement a small percentage, say from 5% to 10% of an unctuous material such as graphite or talc, the purpose of this being to act as a lubricant to aid in the spreading 65 of the cement on the face of the mold.

The facing produced on the refractory lining possesses the property of being fused by the heat of the molten metal after the latter has been introduced into the mold and has distributed itself over the body thereof, the 70 fusion of the cement to the metal causing the casting or pipe to retain a large portion of the same on the finished casting as a protective coating which displays great resistance to corrosion and which may be used to 75 displace the ordinary tar or other coatings according to present practice. Fig. 2 of the drawings shows the refractory mold after a casting operation has taken place, and shows 80 the hollow metal casting 16 provided with the outer coating 17 of the cementitious material. It is well known that cement inhibits corrosion in all iron products, and I have empirically demonstrated that the fused cement coating on the outer surface 85 of the casting materially contributes to its power of resistance to corrosion. It may be noted that because of the highly non-conducting character of the cement facing on the sand lining, that the sand is prevented 90 from attaining sufficient temperature during the casting operation to fuse with the cement so that the cement coated pipe easily cleaves from the mold. Although I prefer to employ the moist sand lining mixture 95 above described with the natural cement facing for producing the coated casting, it will be understood that other sand lining mixtures may be used to yield satisfactory results.

The practice of my method and the making of protectively faced centrifugal castings will in the main be fully understood from the above detailed description thereof. Besides facilitating the casting process, producing an efficient mold and a coated metal product, I have found that with my method a cheap metal mixture may be employed, such for instance as a mixture having the elements phosphorus, carbon, silicon, manganese and sulphur reduced to low values and the costly silicon content reduced from about  $1\frac{1}{2}\%$  down to about  $\frac{7}{10}\%$ , this being materially lower than the silicon content employed in metal mixtures with other processes. It will therefore be seen that the practice of my method is generally characterized by the ease of practicing the same, the efficient mold produced, the desired casting product obtained, and the inexpensive metal mixture used.

While I have disclosed the preferred form of my invention, it will be apparent that numerous changes may be made therein without departing from the spirit of the invention, defined in the following claims.

I claim:

1. In the art of centrifugally casting metal bodies, the method of making a hollow metal casting with an outer protective coat-

- ing fused to the body thereof, which consists in coating a refractory moist rotary mold with a powdered material having the property of absorbing moisture from the mold and of setting to form a fusible facing, and in pouring molten metal into the mold. 5
2. In the art of centrifugally casting metal bodies, the method of making a hollow metal casting with an outer protective coating united to the body which consists in coating the inner wall of a rotary refractory moist mold with a substance for forming a fusible facing, and in pouring molten metal into the mold. 10
- 15 3. In the art of centrifugally casting metal bodies, the method of making a hollow metal casting with an outer protective coating united to the body which consists in coating the inner wall of a rotary refractory moist mold with a cementitious substance which sets to form a fusible facing, and in pouring molten metal into the mold. 20
4. In the art of casting metal bodies, a method of making a hollow metal casting with a protective coating which consists in coating a refractory moist mold with a powdered material having the property of absorbing moisture from the mold and setting to form a fusible facing, and in pouring molten metal into the mold. 25
5. In the art of casting metal bodies, a method of making a metal casting with a protective coating which consists in coating a green sand mold with a powdered material having the property of absorbing moisture from the mold and setting to form a fusible facing, and in pouring molten metal into the mold. 30
- 35 6. In the art of casting metal bodies, a method of making a metal casting with a protective coating which consists in coating a refractory moist mold with a powdered material having the property of absorbing moisture from the mold and setting to form a membranous fusible facing, and in pouring molten metal into the mold. 40
- 45 7. In the art of casting metal bodies, a method of making a metal casting with a protective coating which consists in coating a refractory unbaked mold with a cementitious substance having the property of taking a quick initial set to form a membranous and fusible facing, and in pouring molten metal into the mold. 50
- 55 8. In the art of casting metal bodies, a method of making a metal casting with a protective coating which consists in coating a refractory unbaked mold with a powdered cementitious substance to form a fusible facing, and in pouring molten metal into the mold. 60
- 65 9. In the art of casting metal bodies, a method of making a metal casting with a protective coating which consists in coating a refractory unbaked mold with natural cement to form a fusible facing and pouring molten metal into the mold. 70
10. In the art of casting metal bodies, a method of making a metal casting provided with a protective coating which consists in coating a refractory unbaked mold with a powdered natural cement to form a fusible facing and pouring molten metal into the mold. 75
11. In the art of casting metal bodies, a method of making a metal casting with a protective coating which consists in coating a refractory unbaked mold with a powdered mixture of a cement and a lubricant to form a fusible facing on the surface of the mold and in pouring molten metal into the mold. 80
12. In the art of casting metal bodies, a method of making a metal casting with a protective coating which consists in coating a refractory unbaked mold with a mixture of natural cement and a lubricant to form a fusible facing on the surface of the mold and in pouring molten metal into the mold. 85
13. In the art of casting metal bodies, a method of making a metal casting with a protective coating which consists in coating a green sand mold having a moisture content of from 7% to 11% with powdered natural cement to form a fusible facing, and in pouring molten metal into the mold. 90
14. In the art of casting metal bodies, the method of making a metal casting with a protective coating which consists in coating a green sand mold having a moisture content of from 7% to 11%, with a substance having a property of absorbing moisture from the mold and setting to form a membranous fusible coating. 100
15. In the art of casting metal bodies, a method of making a metal casting with a protective coating which consists in coating a refractory unbaked mold with a mixture of natural cement and an unctuous material to form a skin-like fusible facing in the surface of the mold, and in pouring molten metal into the mold. 105
- 110 16. In the art of centrifugally casting ferrous metal pipe, a method of providing a protective coating for the pipe which consists in coating a green sand mold with a powdered material having the properties of absorbing moisture from the mold and setting to form a fusible facing, and in pouring molten ferrous metal into the mold. 115
17. A metal casting provided with a protective coating composed of natural cement. 120
18. A metal casting provided with a protective coating composed of natural cement and an unctuous material. 125
19. A metal pipe provided with an outer protective coating composed of natural cement fused thereto. 130
20. A centrifugally cast pipe provided on its outer face with a protective coating fused to the body of the casting. 130

21. A centrifugally cast pipe provided on its outer face with a protective cementitious coating fused to the body of the casting. 16
22. A centrifugally cast pipe provided on 5 its outer face with a protective coating composed of a cement and an unctuous material fused to the body of the casting. 20
23. A metal casting provided with a protective coating composed of a substance obtained from the calcination of an argillaceous limestone. 10
24. A ferrous pipe casting composed of a metal mixture having a silicon content of from  $\frac{7}{10}\%$  to  $1\frac{1}{2}\%$  and provided with a protective coating on its outer surface composed of a substance obtained by the calcination of an argillaceous limestone. 15
25. A ferrous pipe casting composed of a metal mixture having a silicon content of from  $\frac{7}{10}\%$  to  $1\frac{1}{2}\%$ . 20
26. A centrifugally cast ferrous pipe composed of a metal mixture having a silicon content of from  $\frac{7}{10}\%$  to  $1\frac{1}{2}\%$ . 25

Signed at New York city, in the county of New York and State of New York this 25 21st day of Feb., A. D. 1923.

WILLIAM D. MOORE.